

Oct. 19, 1937.

G. W. CUPIT, JR

2,096,449

CUTTING AND DRAWING OIL

Filed April 20, 1934



INVENTOR

George W. Cupit, Jr.

BY *John D. Smith*

ATTORNEY

## UNITED STATES PATENT OFFICE

2,096,449

## CUTTING AND DRAWING OIL

George W. Cupit, Jr., Woodside, N. Y., assignor  
to General Chemical Company, New York,  
N. Y., a corporation of New York

Application April 20, 1934, Serial No. 721,454

5 Claims. (Cl. 87—9)

This invention relates to improvements in the art of cutting and drawing metals and to oils for such purposes. More particularly, the invention is directed to cutting and drawing oils comprising 5 sulfur bearing oils derived from sludges formed in oil refining processes in which sulfuric acid is employed.

The principal object of the invention is directed to improvements in the cutting of metals and to 10 the provision of high sulfur cutting and drawing oils and/or cutting and drawing oil bases for this purpose. The invention also aims to provide sulfur cutting and drawing oils or bases light in color and light bodied, and having a high sulfur content 15 substantially all of which sulfur is in chemical combination. It is a further object of the invention to provide high sulfur cutting and drawing oils which are stable and do not become turbid, or deposit sulfur on standing.

20 In oil refining processes, involving treatment of petroleum distillate oils with sulfuric acid, large quantities of sludges are produced. When destructively decomposed by heating, these sludges form gas mixtures containing water vapor and 25 condensable hydrocarbon vapors, and gases such as sulfur dioxide, carbon dioxide, nitrogen and uncondensable hydrocarbons.

It has been discovered that when sludge material, resulting from treatment with sulfuric acid 30 of relatively light hydrocarbon oil distillates containing substantial quantities of sulfur compounds, is dissociated preferably by destructive decomposition by heating to form a hot gas mixture containing hydrocarbon vapors and the gas 35 mixture is cooled, for example to about normal temperature, an oily condensate is obtained which is a sulfur bearing oil possessing properties sought for in cutting and drawing oils. It has been discovered that these oils are light colored, light 40 bodied, stable oils, high in sulfur in strong chemical combination, and which do not become turbid or deposit free sulfur on standing.

A further appreciation of the objects and advantages of the invention may be had from a 45 consideration of the following description of the improved cutting and drawing oils and of methods for making the oils. The accompanying drawing illustrates diagrammatically apparatus by which the improved cutting oils may be made.

50 Referring to the drawing, 10 indicates the combustion chamber of a furnace adapted to burn coal, coke, oil, natural gas or other fuel. Mounted in chamber 10 is a decomposing kiln or retort 11 of any desirable construction, for example a fixed shell provided with suitable mechanism such

as a screw conveyor, not shown, to facilitate discharge of coke. A rotary retort may also be employed if desired. Preferably an externally heated kiln adapted to substantially exclude admission of air is used. One end of kiln 11 5 communicates with a gas outlet 13, and the opposite end projects into a header 14 into which the solid residue of the decomposition of the acid sludge is continuously discharged. Header 14 empties into air-lock 15 through which coke may 10 be discharged without admitting air to the kiln. Acid sludges constituting sources of the improved cutting oils are run into the kiln from supply tank 17 through a valve-controlled pipe 18. Gas outlet 13 is connected to the lower end of a cooler or 15 condenser 20 of any suitable construction, either air or water cooled, and operated so as to reduce the temperature of the gas stream to substantially normal to condense the bulk of the water vapor and a major portion of condensable hydrocarbons 20 contained in the gas. Condensate from the cooler drains into a collecting tank 21 through a pipe 22 having a liquid seal.

The gases uncondensed in cooler 20, containing principally sulfur dioxide, are discharged 25 through gas line 23, and may be used as desired, for example, in the manufacture of sulfuric acid.

Separator 21 may be a tank or vat large enough 30 to permit continuous gravity separation of water and oil contained in the condensate discharged from condenser 20. The hydrocarbon oils of the condensate rise to the top of the mass in the separator, and may be withdrawn continuously or intermittently through pipe 25 discharging into a collecting tank 26. Water settling to the bottom 35 of the separator may be drawn off through pipe 27, controlled by valve 28, and discharged to waste or otherwise disposed of.

The still 30, of any approved construction, may be externally heated by hot combustion gases 40 generated in brickwork setting 31. Raw condensate from collecting tank 26 is run into the still through pipe 38, controlled by valve 39. Vapors generated in the still flow through line 41 to a condenser 43, the condensate of which drains 45 through pipes 45 and 46, into receivers 50 and 51.

Cutting oils of the invention may be made in apparatus such as illustrated in the drawing and described above by operating substantially as follows:

In producing the improved cutting oils, acid sludges which may be employed are those resulting from sulfuric acid treatment of light distillate oils obtained from petroleum crudes containing sulfur. The acid sludges employed in making 55

the cutting oils of the present invention are preferably sludges resulting from treatment with sulfuric acid of light hydrocarbon oil distillates such as gasoline and kerosene, containing preferably not less than about 0.15% sulfur, although 5 distillates containing less sulfur may be employed if desired. Illustrative examples of distillate oils from which sludges are produced of a character suitable for use in the present invention 10 are straight-run gasoline distillates containing about 0.15% sulfur or more, and cracked distillates averaging 0.25 to 0.30% sulfur or more.

Sludge material, of the type indicated and 15 which may have a titratable acidity of 40% to 60% expressed as  $H_2SO_4$ , is continuously fed into kiln 11 from supply tank 17. The burners in furnace 10 are adjusted to preferably maintain within the kiln temperatures desirably not in excess of about 750° F., as above this temperature 20 the sulfur oils of the present invention tend to be decomposed. The preferred temperatures are about 250° F. at the sludge inlet end, and about 500 to 600° F. at the coke outlet end of the kiln.

The sludge, gradually passed through the 25 retort, is relatively gradually heated through the preferred temperature range and is dissociated by the action of heat, and the free and combined sulfuric acid of the sludge is reduced to sulfur dioxide by the hydrogen of the hydrocarbons 30 and/or by the carbonaceous matter contained in the sludge. The sludge material is thus dissociated, as by the destructive decomposition method indicated, with production of water vapor, and hydrocarbon vapors and sulfur compounds are formed. Residual coke is continuously 35 discharged from the kiln through air-lock 15. The major part of the sulfur oils of the present invention are evolved by the time the sludge has reached a temperature of 350-400° F.

40 The gas resulting from the decomposition of the sludge contains principally water vapor and sulfur dioxide, substantial amounts of condensable hydrocarbons and sulfur compounds and smaller quantities of uncondensable hydrocarbons and gases such as carbon dioxide, carbon monoxide, and nitrogen. For example, the exit 45 gas mixture of the retort may contain by volume about 50% water vapor, about 10% condensable hydrocarbon vapors and sulfur compounds, the balance comprising sulfur dioxide, carbon dioxide, carbon monoxide, nitrogen, hydrocarbon gases and oxygen. As previously noted, according to a preferred embodiment of the process for 50 making the cutting oils of the invention, decomposition of sludges is effected in the kiln substantially in the absence of oxygen. When so operating, formation of carbon dioxide is lessened, presumably because oxidation of hydrocarbons and burning of carbonaceous matter of the sludge 55 is prevented.

The hot gaseous and vaporous products of decomposition of the sludge are discharged from the kiln and passed through conduit 13 into condenser 20 in which the gases are cooled to substantially normal temperatures. Cooling may be accomplished by circulating through the condenser in indirect heat exchange relation with the retort gas mixture any suitable cooling liquid or gas. In place of the condenser illustrated in 70 the drawing, a vertical tower having a spray head at the top for introduction of water may be employed. In such cases, the retort gas mixture is introduced into the bottom of the tower and flows upwardly, intimately contacting and 75 mingling with the downwardly directed spray of

water fed in at the top of the tower. The amount of cooling water introduced is so controlled as to cool the exit gases leaving the top of the tower to about normal atmospheric temperatures.

During cooling of the retort gas mixture in the condenser 20, substantially all of the water vapor and the major portion of the condensable hydrocarbon vapors and sulfur compounds are condensed out of the gas stream. The condensate 10 of cooler 20, containing varying proportions of water and liquid hydrocarbons and sulfur compounds, is drained through pipe 22 into separator 21. In the latter, the oils rise to the top of the liquid mass in the tank, and may be intermittently or continuously withdrawn through pipe 25 into tank 26 for collecting what may be considered a raw condensate. The water settling to the bottom of the separator 21 may be discharged 15 from the system through pipe 27.

The oil collecting in tank 26 is an oil containing generally from about 3 to about 22% sulfur, apparently in strong chemical combination. It will be understood the sulfur content of this condensate may vary considerably in accordance with the characteristics of the initial crude oils and of the acid sludges produced on treatment of the hydrocarbon oil distillates with sulfuric acid. For example, an acid sludge formed through sulfuric acid treatment of a 30 straight-run gasoline yielded an oil condensate of 12% by volume of the sludge, the condensate analyzing 14.8% sulfur. A cracked distillate sludge yielded 10% by volume of oil condensate having a sulfur content of 7.5%. In another instance, a cracked distillate averaging about 0.25 to 0.30% sulfur produced on treatment with sulfuric acid a sludge which, on treatment in accordance with the present method, yielded 10.8% by volume of oil condensate analyzing 20.8% 40 sulfur.

By the present invention, it has been found that oils produced as described above are sulfur-containing oils having properties rendering them particularly suited for use as cutting and drawing oils. The raw condensate recovered in tank 26 may, if desired, be used directly as a cutting or drawing oil. However, since the oil in this state contains substantial quantities of foreign matter, such as coke dust and tars, and also a low boiling fraction of low flash point it is preferred to remove these substances. This may be done by distillation. For this purpose oils from tank 26 are run into still 30 through line 38. The distillation operation may be carried out in any suitable still, preferably one provided with equipment for collecting separate fractions of distillate. Distillation of the raw condensate is principally for two purposes, first, to remove coke and tars from the oil, and second, to produce preferably two fractions, one having a relatively low boiling range and containing low flash point hydrocarbons and another fraction having a higher boiling point range and constituting the preferred cutting and drawing oil of the invention. Distillation may be effected for example by external heating of still 30. If desired, distillation of the crude condensate may also be accomplished at temperatures lower than those hereinafter mentioned by introducing 55 live steam directly into the oil body while externally heating the same. Distillation may also be effected, though possibly less desirably, by superheated live steam, using steam at slightly above atmospheric pressure and heated to say 225-250° F. 70 75

before introduction into the oil. Vacuum distillation may be employed if desired.

Still 30 is operated to produce a first cut including all the oils distilling over at temperatures up to about 350° F. Vapors generated within this temperature range are liquefied in condenser 43, and are run into receiver 50. This relatively low boiling fraction may for example constitute approximately 20% by volume of the raw condensate.

0 fed into still 30. When removal of these low boiling fractions from the oil in still 30 is substantially complete, the temperature is raised to distill over oils having boiling points ranging from about 350° F. up to about 650° F. Vapors formed 15 are condensed in cooler 43, and may be recovered in receiver 51. This high boiling fraction may comprise for example about 70% by volume of the raw condensate introduced into still 30. Approximately 10% of the original raw condensate 20 withdrawn from tank 26 remains as a coke or asphalt residue in the still.

The low boiling cut recovered in receiver 50 contains a slightly higher percentage of sulfur than the higher boiling fraction collected in receiver 25 51. This low boiling cut while useful as a cutting oil has somewhat too low flash point for general use in cutting.

The preferred cutting and drawing oil of the invention is the higher boiling fraction recovered in receiver 51, and such oil may be so used directly as condensed in cooler 43. The oil, however, apparently contains substances such as pyridines and mercaptans somewhat unstable on standing. Accordingly, it is preferred to further treat the oil 35 to stabilize the same and remove odors. This may be accomplished by treating the oil with a solution of caustic soda or sulfuric acid or both. When employing caustic alkali, as is preferred, the oil may be agitated with a 20% caustic soda 40 solution at temperatures of about 190° F. until reaction appears complete. The reaction products are allowed to settle, and are withdrawn. The oil may then be washed with water to remove traces of alkali, and brightened as by blowing with 45 air, or other methods.

The oil may be stabilized by treatment with sulfuric acid, say about equal volume, and washed with water and alkali to remove traces of acid. It is preferred to use acid of concentration not in 50 excess of about 60%  $H_2SO_4$ , since acid of this or less concentration, does not appear to have any appreciable effect on valuable sulfur compounds which should preferably be retained in the product. If desired the oils may be stabilized by using acid of greater concentration, say up to about 55 93%  $H_2SO_4$ , in which case the amount of stronger acid employed should not desirably exceed about 7% by volume of the oil treated.

Treatment of the oil with either caustic alkali 60 or sulfuric acid notably improves the odor and increases the stability of the oil. In some instances, it is preferred to subject the oil to treatment with both caustic alkali and sulfuric acid. In this case, after subjecting the oil to the caustic 65 soda treatment noted above, and removing the alkali extract, the oil is washed with water to remove the alkali, and is then treated with one or more washes of equal volume of dilute sulfuric acid, for example 30%  $H_2SO_4$ . The final oil product may 70 be washed with water to remove traces of acid, and then brightened by blowing with air.

Strong sulfuric acid appears to extract at least some of the valuable sulfur compounds from both the stabilized and unstabilized oils of the invention. It has been found in this connection that

sulfuric acid stronger than about 70% and preferably about 93.2% (66° Bé.) will remove these sulfur compounds from the stabilized and unstabilized oils to form an acid sludge, and on hydrolysis of the acid sludges produced by such treatment practically the same volume of oil is recovered as was removed with the sulfuric acid and the oils recovered on hydrolysis are considerably higher in sulfur content than the original oil. For example, on treating a heavy fraction stabilized by treatment with both caustic alkali and weak sulfuric acid, boiling approximately within the range 350-650° F. and containing about 11.6% sulfur, with about twice the volume of 93.2% sulfuric acid (66° Bé.), the sulfur in the acid 10 treated oil, after separation of the acid sludge formed was reduced to about 1.9%, and the sulfur content of the oil obtained after hydrolysis of the acid sludge was about 19%.

The heavy fraction stabilized, for example as 20 mentioned above, is a sulfur bearing mineral oil, light in color, light bodied, possessing no undesirable odor, and having a high sulfur content, substantially all of which is in strong chemical combination. It appears substantial amounts of 25 the contained sulfur are present as alkyl sulfides and possibly also some disulfides. The sulfur content varies from about 3 to about 22%. The oil on standing does not become turbid or deposit sulfur, a property highly desirable in a cutting 30 oil. In this connection, sulfur oil of the invention has been subjected to a cold test, and it was found that at a temperature of 14° C. below zero, there is no separation of sulfur, the oil remaining unclouded and of substantially un- 35 changed viscosity.

The oils of the invention are a light straw color, a feature which is particularly advantageous since there is no tendency for the oil to hide the work from observation during the cutting process. The specific gravity of a representative oil is about 0.98. The viscosity is low, about 32 to 34 Saybolt at 100° F. This is a material advantage in cutting and drawing operations. Prior cutting and drawing oils and bases 40 are generally of high viscosity, and dilution with lighter oils is necessary to produce an oil having a viscosity suitable for working conditions. This dilution results in an oil having a lowered sulfur content. The oils of the invention are light 45 50 bodied, flow easily and spread well, and hence may be used directly as cutting and drawing oils if desired. Further, since the oils are readily miscible with heavier oils in all proportions and as the sulfur content is high, the base oils of the 55 invention may be compounded with non-sulfur mineral oils of requisite viscosity if desired to give compositions of desired characteristics and of high sulfur content.

As observed the oils of the invention may be 60 used directly as cutting and drawing oils, or may be diluted with oils such as mineral or lard oil. In one instance, a hard chrome-manganese steel (6150 S. A. E. steel) was cut leaving a smooth, polished surface, using a cutting oil comprising 65 a 14% sulfur-bearing oil of the invention (stabilized heavy fraction) diluted with an equal volume of a mixture of 600 W. and a heavy cylinder oil. Satisfactory results were also obtained when cutting the same grade of steel using the same 70 14% sulfur bearing oil in combination with other mineral oils in the following proportions: stabilized oil 20%, 28° Bé. paraffine oil 18%, heavy cylinder oil 62%; stabilized oil 16%, 28° Bé. paraffine oil 30%, heavy engine oil 54%; stabilized oil 75

10%, 28° Bé. paraffin oil 90%; stabilized oil 33%, D. T. E. extra heavy lubricating oil 45%, 600 W. 22%; stabilized oil 10%, D. T. E. extra heavy lubricating oil 30%, 28° Bé. paraffin oil 60%.

5 I claim:

1. A cutting and drawing oil base comprising a relatively light-bodied, light-colored, low viscosity sulfur oil, boiling at temperatures less than about 650° F., stable at low temperature with respect to sulfur deposition, substantially free of free sulfur, containing alkyl sulfides, having a sulfur content not less than about 7.5% and not more than about 22% and formed by dissociating sludge material, resulting from sulfuric acid treatment of hydrocarbon distillate oils obtained from sulfur-containing crudes, with aid of heat to break up the sludge and under conditions to form a hot gas mixture containing water and hydrocarbon vapors, cooling the gas mixture to form a condensate comprising water and oil boiling at temperatures less than about 650° F., separating oil and water, and recovering the oil.

2. A cutting and drawing oil base comprising a relatively light-bodied, light-colored, low viscosity sulfur oil, boiling substantially within the range 350° F. to 650° F., stable at low temperature with respect to sulfur deposition, substantially free of free sulfur, containing alkyl sulfides, having a sulfur content not less than about 7.5% and not more than about 22% and formed by dissociating sludge material, resulting from sulfuric acid treatment of hydrocarbon distillate oils obtained from sulfur-containing crudes, with aid of heat to break up the sludge and under conditions to form a hot gas mixture containing water and hydrocarbon vapors, cooling the gas mixture to form a condensate comprising water and oil, separating oil and water, distilling the oil, and recovering as condensate a fraction boiling substantially within the range 350° F. to 650° F.

3. A cutting and drawing oil base comprising a relatively light-bodied, light-colored, low viscosity sulfur oil, boiling at temperatures less than about 650° F., stable at low temperature with respect to sulfur deposition, substantially free of free sulfur, containing alkyl sulfides, having a sulfur content not less than about 7.5% and not more than

about 22% and formed by dissociating sludge material, resulting from sulfuric acid treatment of light hydrocarbon distillate containing not less than about 0.15% sulfur, with aid of heat to break up the sludge and under conditions to form a hot gas mixture containing water and hydrocarbon vapors, cooling the gas mixture to form a condensate comprising water and oil boiling at temperatures less than about 650° F., separating oil and water, and recovering the oil.

4. A cutting and drawing oil base comprising a relatively light-bodied, light-colored, low viscosity sulfur oil, boiling substantially within the range 350° F. to 650° F., stable at low temperature with respect to sulfur deposition, substantially free of free sulfur, containing alkyl sulfides, having a sulfur content not less than about 7.5% and not more than about 22% and formed by dissociating sludge material, resulting from sulfuric acid treatment of light hydrocarbon distillate containing not less than about 0.15% sulfur, with aid of heat to break up the sludge and under conditions to form a hot gas mixture containing water and hydrocarbon vapors, cooling the gas mixture to form a condensate comprising water and oil, separating oil and water, distilling the oil, and recovering as condensate a fraction boiling substantially within the range 350° F. to 650° F.

5. A cutting and drawing oil base comprising a relatively light-bodied, light-colored, low viscosity sulfur oil, boiling at temperatures less than about 650° F., stable at low temperature with respect to sulfur deposition, substantially free of free sulfur, containing alkyl sulfides, having a sulfur content not less than about 7.5% and not more than about 22% and formed by dissociating sludge material, resulting from sulfuric acid treatment of hydrocarbon distillate oils obtained from sulfur-containing crudes, with aid of heat to break up the sludge and under conditions to form a hot gas mixture containing water and hydrocarbon vapors, cooling the gas mixture to form a condensate comprising water and oil, separating oil and water, distilling the oil, and recovering as condensate oil boiling at temperatures less than about 650° F.

GEORGE W. CUPIT, JR.